

# UNITED STATES PATENT OFFICE.

RICHARD D. DIVINE, OF CHICAGO, ILLINOIS.

## PROCESS OF SEPARATION OF METALS.

No. 921,372.

Specification of Letters Patent.

Patented May 11, 1909.

Application filed November 12, 1906, Serial No. 343,085. Renewed September 17, 1908. Serial No. 458,505.

To all whom it may concern:

Be it known that I, RICHARD D. DIVINE, citizen of the United States, residing at Chicago, in the county of Cook and State of Illinois, have invented new and useful Improvements in Processes of Separation of Metals, of which the following is a specification.

This invention is a process for the separation of zinc from lead and antimony oxids, 10 and the reduction of the metal oxids to the metallic state.

The invention is supplemental to, and an improvement of, the Parke's process for the reduction of metals. In the Parke's process, for extracting precious metals from lead, zinc is added to molten lead containing gold, silver and copper, and these metals form an alloy with the zinc by reason of their greater affinity for the zinc than for the lead, and this 15 alloy is lighter than lead and rises to the top, carrying the precious metals with it, whence it can be removed by skimming. These skimmings are further treated for the separation of the zinc therefrom and the recovery 20 of the precious metals, the zinc being driven off by heat and again used for another operation. But before the zinc which is added to the bullion has any action on the silver it has been found that a certain amount is necessary to "saturate" the lead, and the zinc so used remains with the desilverized lead, and does not skim off, and hence it is necessary 25 to give said lead another treatment to free it from the saturating zinc. To do this it is heated with an oxidizing flame or steam is blown through it. This method will oxidize the zinc together with a small amount of the lead and antimony, leaving the lead free from zinc and antimony, and forming oxids of 30 these metals, which rise to the top and are skinned off. My process relates to the separation of the metals in these oxids or skimmings. The skimmings or oxids are first cooled and then crushed, and to the crushed 35 product is added carbonate of soda in the proportion of two hundred pounds to one ton of the oxids, and there is also added pulverized oil cake in the proportion of one hundred pounds to the ton. These are thor- 40oughly mixed and placed in a suitable retort and heated to a temperature which will expel the zinc which volatilizes at a lower heat than the lead and antimony. The heat is therefore not intense enough to remove the lead 45 and antimony, but by the action of the carbonate of soda and oil cake said oxids are re-

duced to a metallic state. The zinc is then easily driven off, and is condensed and collected in a suitable room as commercial zinc oxid.

60

The carbonate of soda greatly assists the reduction in consequence of its dissolving and decomposing effect, and it generally facilitates the action. There is very little residue thereof after the zinc is driven off, 65 and it is evident that the sodium carbonate is decomposed. Its action is probably as follows: The hot carbon acts upon the sodium carbonate, producing by its reduction a certain amount of sodium which by its 70 strong attraction for oxygen combines with that contained in the metallic oxids. In the reaction carbonic acid is formed, and this acting upon the vapors of zinc assists somewhat in the oxidization of the volatile zinc. 75 The reaction may be written as follows:



then



80

This cake has many advantages for the purpose. It is essentially pure carbon and leaves practically no residue when burned in a current of air or oxygen, and it is this fact 85 which makes it more valuable than coal, charcoal or coke, all of which leaves ashes or deposits which would have to be gotten rid of.

The action of the oil cake and carbonate of soda is to reduce the oxids to the metallic 90 state, and by simply keeping the charge in the molten condition at a low heat the zinc is volatilized and again oxidized while the lead and antimony remain behind as metals practically free from impurities. Air is ex- 95 cluded to a great extent from the retort as it would be liable to again oxidize the lead and antimony, and the temperature is kept low for the same reason. The extraction of the zinc by this method is practically per- 100 fect, and the reduced lead and antimony contain only a small percentage of zinc, and are free from any deposit of silica or ashes which would result from the use of coal or the like.

105

Heretofore, the zinc oxid in the skimmings referred to has been lost, as there has been no way of extracting it from the oxids of lead and antimony and saving it. This resulted in a certain expense which the present invention 110 saves. Also the presence of the other oxids has been a nuisance in clogging the smelting

furnace by forming deposits on the sides which retain other metals, fluxes, etc. and gradually make the furnace smaller and curtail the output. Even with its disadvantages it has hitherto been cheaper to lose the zinc than to try to extract it, but by the use of a cheap reducing agent such as oil cake and the process above described, the reduction and separation can be made at a substantial saving.

I claim:

The process of separating the oxids of

lead, antimony and zinc, consisting in mixing said oxids with oil cake and sodium carbonate, and heating said mixture sufficiently to reduce the oxids to the metallic state and vaporize the zinc.

In testimony whereof I have signed my name to this specification in the presence of two subscribing witnesses.

RICHARD D. DIVINE.

Witnesses:

LEWIS M. RANDOLPH,  
JOHN McCABE.